

Dec. 25, 1934.

E. J. MAUST

1,985,868

MANUFACTURE OF CEMENT

Filed Oct. 21, 1931

3 Sheets-Sheet 1



FIG. 1.



INVENTOR  
ERNEST J. MAUST  
BY *Arthur M. Macarthur*  
ATTORNEY

Dec. 25, 1934.

E. J. MAUST

1,985,868

MANUFACTURE OF CEMENT

Filed Oct. 21, 1931

3 Sheets-Sheet 2

SHALE LIME STONE



INVENTOR  
ERNEST J. MAUST.  
BY *Arthur Richardson*  
ATTORNEY

Dec. 25, 1934.

E. J. MAUST

1,985,868

MANUFACTURE OF CEMENT

Filed Oct. 21, 1931

3 Sheets-Sheet 3

FIG. 3.



FIG. 4.



INVENTOR  
ERNEST J. MAUST  
BY *Arthur Richardson*  
ATTORNEY

## UNITED STATES PATENT OFFICE

1,985,868

## MANUFACTURE OF CEMENT

Ernest J. Maust, New York, N. Y., assignor to The Dorr Company, Inc., New York, N. Y., a corporation of Delaware

Application October 21, 1931, Serial No. 570,111

6 Claims. (Cl. 106—25)

The present invention relates to the manufacture of Portland cement, with special reference to a method of and apparatus for controlling the composition of the mixture of raw constituents as prepared by what is known as the wet process.

Since the raw materials used in the manufacture of cement, such as limestone and shale, are obtained from quarries or natural deposits, there is usually a considerable variation in chemical composition of materials obtained from different areas or different strata of the quarry, and while preliminary chemical control may therefore be effected in a general way by selective quarrying, such control is at most a very rough approximation and must be followed by suitable correction at another step or steps in the process.

Heretofore the necessary correction has been made by running the ground mixture from the mills into batch slurry mixers or correction tanks from which catch samples are taken and analyzed. Two or more such tanks thus filled and tested, are maintained with high lime and low lime mixtures which are drawn off in suitable proportions into kiln feed basins to form the proper mix for burning. Such correction tanks require from six to eight hours filling time, which together with the time required for sampling and analyzing results in a lapse of ten or twelve hours from the time the raw materials for that batch entered the mills, with the disadvantage that such analysis lags much too far behind the mill feed to permit of any but a very general control by variation of the composition of mill feed.

The chief object of the present invention is to obviate this disadvantage and provide a substantially continuous and more accurate control of the composition of the mixture throughout the process. This object is accomplished through the utilization of closed circuit grinding with repeated analysis of the mill output at relatively short periods, two hours or less, while repeatedly correcting the mill feed to compensate for variations from the desired mixture as indicated by such analyses and thus cause the composition of the mill output to average that desired; together with the use of a thickener in a manner to receive and continuously blend the fluctuations in composition of the mill output whereby even relatively wide fluctuations if of sufficiently short duration and properly average or compensated, will be smoothed out in the thickener underflow. Further correction of the thickener underflow is obtained through the practice of what may be termed closed circuit thickening, which comprises recirculating a portion of the underflow through

the thickener, advantage being taken of the variation of mixture within different parts of the thickener by recirculating a portion of the underflow via a zone in the thickener containing a mixture rich in the constituent needed for correction. The amount of variation necessary for correction is slight because variations in the thickener underflow take the form of a relatively slow trend in which the time required for a variation sufficient to necessitate correction is inclusive of a period sufficient for the making of several analyses of the underflow.

A modification of the invention accomplishes this object of continuous and accurate control, through the use of closed circuit grinding in combination with a plurality of thickeners arranged to cooperate with each other in the correction of fluctuations in composition of the mill output. To this end variations of mixtures discharged from the grinding circuit rich in lime are blended or averaged separately from the variations of mixtures deficient in lime, in high and low lime thickeners, respectively, and final adjustment effected by proportionate blending of the underflow from the different thickeners according to the analyses of such underflows. There may be several high-lime and several low-lime thickeners to provide a number of grades of each of the two kinds of mixtures for final adjustment. There may also be one or more medium thickeners for receiving substantially correct or medium mixture, or for receiving mutually compensating fluctuations in mixture of such short duration as to readily blend into an average which will equal or approximate the desired composition.

In distributing the mill output to the different thickeners it may be diverted substantially all to one thickener at a time, or split among two or more thickeners in portions differing according to the kind of mixture being delivered at the time and the difference in kind of average mixture to be stored in each of such thickeners.

For final correction of the slurry to bring it to the proper complex ratios and fine adjustment of lime ratio before going to the filter or kiln, it is passed through a plurality of correction tanks connected in series and supplied with the slurry and the necessary correction materials in a manner enabling the slurry to be detained and sampled, and further corrected if necessary, at successive points en route to the filter or kiln without interruption to continuity of supply to the filter or kiln.

Other objects and advantages of the invention will be apparent from a perusal of the following

5

10

15

20

25

30

35

40

45

50

55

specification and the drawings accompanying the same.

In the drawings:

Fig. 1 is a diagram of a combination and arrangement of apparatus elements for carrying out the invention through the use of a single, large equalizing thickener.

Fig. 2 is a modified arrangement using a plurality of small thickeners for separate averaging and thickening of high lime and low lime mixtures.

Fig. 3 is a flow sheet illustrating the method of proportioning the thickener feed between high lime and low lime thickeners.

Fig. 4 is a flow sheet showing the method of proportioning the thickener feed among high lime, low lime and medium mixture thickeners.

Referring to the drawings in detail, and first to Fig. 1, bins 1 and 2 are for storing the main raw material such as crushed cement rock or limestone for ready supply to a primary or coarse grinding ball mill 3, as indicated by the flow line 4. The rock, roughly classified, is stored in the bins 1 and 2 as high lime and low lime rock, respectively, suitable feed control means, such as the usual variable speed feeders, indicated at 5 and 6, being operatively connected between each bin and the mill for proportioning the materials fed to the mill. The primary mill 3 is arranged in closed circuit with a Dorr classifier 7, from which the overflow is fed into the bowl 8 of a Dorr bowl classifier 9 as indicated by the flow line 10. Suitable means are provided for adding water to the mill and classifier as indicated at 11 and 12 to maintain optimum working dilutions. Where the raw material taken from the bins 1 and 2 contains a considerable quantity of natural fines, it may be introduced directly into the primary classifier 7, the raw material being supplied in a size sufficiently small for such method of feed. The bowl classifier 9 is arranged in closed circuit with a secondary or fine grinding mill 13, means being provided for adding water to the bowl 8 of the classifier and to mill 13 as indicated at 14 and 15, and for adding clay or clay slip to the secondary mill 13 as indicated at 16.

The bowl classifier 9 is arranged to discharge the overflow from the bowl 8 into a large Dorr thickener 17 as indicated by flow line 18, a sampler 20 being arranged to take off a sample as indicated by flow line 21. The sampler 20 may be of any known or other suitable type operable to take a composite sample proportional in volume to the volume of flow and for a given length of time. By taking the sample from the flow line 18 between the bowl overflow and the thickener 17, the sampling of the thickener feed is done at a point where the ground mixture is at its greatest dilution and in a turbulent and well dispersed condition.

The thickener 17 is a Dorr type traction thickener of relatively large capacity in proportion to the grinding apparatus to afford a wide margin of storage capacity. It has the usual sloping bottom 22 along which the thickened slurry is raked by the usual rotating rake arms 23 and 24 toward the central discharge point 25 to the underflow line 26. It is also provided with the usual central, annular, feed trough 27 which receives the feed from the bowl 8 as indicated by the flow line 18, and delivers it into the thickener below the liquid level 28, all as is well understood in the art. The thickener overflow 29 may lead to waste or be passed back into circuit in the usual manner as water supply to the grinders or classifiers. A

return feed launder 30 situated near the center is provided with distributing pipes 31, 32 and 33, for conducting the return feed to a zone in the thickener near the discharge 25, a zone near the top of the thickener, and a zone intermediate the discharge opening and the top, respectively. Each of the distributing pipes is provided with a suitable valve means 34, 35 and 36 respectively, for controlling the flow of return feed therethrough.

Underflow from the thickener is conducted by way of pump 37 to a surge tank 38 as indicated by flow line 39, the surge tank 38 discharging through flow line 40 and valves 41 and 42 into two or more slurry mixers 43 and 44, the slurry mixers in turn being arranged to discharge through regulating valves 45 and 46 into an equalizing storage tank 47. From the storage tank the slurry passes on to the usual kilns or other suitable burning means as indicated at 48, either directly or through filters. The surge tank 38 is arranged to discharge also into the return feed launder 30 as indicated by flow line 49. Suitable valve means 50 and 51 are provided in the flow lines 40 and 49, respectively. A sampler 52, preferably of the automatic type, is arranged to take samples of the flow through flow line 40. The apparatus is also arranged to facilitate the taking of samples, such as the usual catch-sample from the surge tank 38 as indicated diagrammatically at 53. Means are also provided for adding suitable correction materials to the contents of the slurry mixers 43 and 44 as indicated at 54 and 55, to effect any final correction necessary.

In the operation of the system and apparatus, shown in diagram in Fig. 1 to carry out the method of the invention, the raw materials, classified into two portions, one of high lime and one of low lime content, for example, the limestone and shale, or limestone with little or no clay and limestone with more clay than that required for a proper mix, and properly crushed for grinding, say about three-fourths inch, are stored in the high lime and low lime supply bins 1 and 2 respectively, according to their lime content, and fed therefrom through the feed regulating means 5 and 6 into the primary mill 3 along with the necessary amount of water supplied through conduit 11 to bring the contents of the mill to the optimum dilution or viscosity for grinding to the size desired. The mill 3 being arranged in closed circuit with the classifier 7, discharges the ground materials thereinto, water being added from the source 12 to bring the dilution from that of the optimum grinding dilution to the further dilution desired for classification. The classifier operates to remove the oversize and return it to the mill 3 as indicated by flow line 57. From the classifier 7, the fines with the bulk of the water, overflow into the bowl classifier 9, from which the intermediate oversize is fed into a secondary or fine grinding mill 13 as indicated by flow line 58, which secondary mill, being in closed circuit with the bowl classifier 9, delivers its discharge into the bowl 8 of the classifier as indicated by flow line 59. Where there is insufficient clay or its equivalent in the raw material supplied from bins 1 and 2, the required amount of clay may be added to the contents of the mill 13 as indicated at 16. Water is supplied by 15 to the mill 13 to bring its contents to the proper viscosity for efficient grinding at the size determined upon. Where the material supplied from the bins 1 and 2 contains a considerable amount of natural fines, the feed therefrom may be run directly into the classifier

7 instead of first into the primary mill, the raw material being crushed to a size somewhat finer than three-fourths inch and more suitable for classifier feed, as will be well understood by those skilled in the art.

8 To bring the feed of the bowl classifier 9 to the proper dilution for final classification, water is added as indicated at 14. At this final and highest dilution the finished fines overflowing the bowl 8 are passed into the annular feed launder 27 of the thickener 17, the mixture being maintained in sufficient turbulence and dispersion on its way past the sampler 20 to the thickener to enable a substantially perfect sample 10 to be taken. Samples are thus repeatedly taken and analyzed to ascertain the composition of the thickener feed. The thickener feed passing into the launder 27 is distributed thereby into the thickener 17 in the usual manner.

15 20 The rake arms 23—24 rotate at the proper speed to rake the settled material into the central discharge point 25 and produce a slight disturbance as hereinafter described, but insufficient to prevent the desired decantation. The thickened discharge or underflow passes on through the underflow line 26 to pump 37 from whence it is passed on through flow line 39 to the surge tank 38. From the surge tank the slurry is conducted 25 on through flow line 40 to one of the batch slurry 30 mixers, say 41, a sample of the slurry being taken at 52. From the slurry mixers 41 and 42 the slurry is drawn into the equalizing storage tank 47, the batch mixers being alternately filled and drawn, one drawn while the other is being filled 35 and its contents tested and corrected to bring it to the final desired adjustment of complex ratios, such as ratios of iron, silica, alumina and soluble salts. From the equalizing tank 47 the slurry is run either directly to a kiln for burning or first 40 through a filter and then to the kiln.

45 As the dilution of the discharge from the secondary mill 13 is only that necessary for optimum grinding, viscosity is relatively low and may be as low as that at which the final raw product is passed to the kiln for burning. It is therefore necessary to further dilute the discharge of mill 13 for hydraulic classification in the bowl classifier 9, which dilution is effected as it is fed into the bowl 8 along with the overflow from classifier 50 7 with additional water supplied at 14. As the dilution at which the desired fines overflow the classifier bowl 8, is the highest dilution attained in the process, and the turbulence and dispersion of the mixture is at a maximum in the flow line 18 55 from the bowl overflow to the thickener, the sampling is done at this point so as to obtain a fair sample of the whole volume of mixture flowing during the taking of the sample. The samples are thus taken at given intervals and for a suitable length of time, the intervals being regulated 60 preferably according to the time required to make an analysis of the composition of a sample, which time for example, may be in the neighborhood of two to four hours, and is sufficient to give the 65 operator a definite accounting of the average being carried in the thickener. This time, however, is small compared with the time of detention in the thickener, whose equalizing effect on any variation in composition of feed is brought to a 70 high degree of perfection by rotating the rake arms at a speed sufficient to properly rake the thickened underflow to the point of discharge with slight stirring, insufficient to prevent the desired decantation or settling, and by having 75 the capacity of the thickener so large in propor-

tion to the rate of feed and intervals of analysis and correction, that the quantities of mixture fed into the thickener during such successive periods are spread in strata sufficiently thin to be intermixed by the slight stirring action of the rake arms. This coordination of magnitudes of time, capacity of settling zone and rate of stirring is an important feature of the invention which makes for the attainment of my object of improved control of the composition of the product.

10 The underflow from the thickener is thus of a composition which is an average of the total volume of mixture fed into the thickener for a long period of time relative to the time between corrections of such mixture, with the result that any 15 change in the composition of the underflow takes the form of a gradual trend requiring a long time, in the neighborhood of several days, to exceed a permissible margin, which makes the taking of ordinary catch samples at 52 sufficient to indicate changes in the trend in time to make suitable correction in thickener feed to offset a trend toward excess. Such offset may be accomplished by making a correction over-compensating for the requirement indicated by the analysis of the 20 catch sample which accelerates the trend in an opposite direction sufficiently to prevent the trend from exceeding the permissible variation.

25 As a specific, practical example of feed control and thickener underflow response, an analysis at 30 intervals of two to four hours gives the operator definite knowledge of what he is grinding and a definite accounting of the average being carried in the thickener. The raw mill feed for one period is roughly adjusted to compensate for discrepancies of the preceding period and the variations between the different periods are permitted to average out in the thickener. Short period variations in the mix going to the thickener 35 do not affect the mix in the thickener discharge except as they affect the average of about 36 hours operation. Even when a distinct and permanent change is suddenly made in the mix to the thickener the swing toward it in the thickener discharge is gradual.

40 In addition to the tendency to variation in different thin strata, due to slight variations in composition of feed for brief intervals of time for making corrections according to the requirements indicated by analysis of the samples of feed, 45 which variations are substantially offset by the slight disturbing effect of the rake mechanism on the relatively thin strata, there is a slight variation in composition at different intermediate zones in the thickener due to difference in settling rate of the different main constituents so that even though the composition of the solid constituents of feed, and consequently the composition of the solid constituents of the underflow are uniform, there will be a zone near the 50 top of the thickener where the composition will be low in lime, an intermediate zone where the composition will be higher in lime and a zone near the discharge where the composition of the thickened mixture will be that of the feed. This 55 will be clear when it is recalled that with an overflow of liquids only, all the solids in the feed will pass out with the underflow so that the composition of the mixture of solids in the underflow will be identical with that of the mixture of solids in the feed, regardless of intermediate stratification due to difference in settling rate of different constituent solids.

60 This intermediate segregation is taken advantage of to bring about a finer and relatively more 65

- rapidly responsive control of the composition of the underflow without having to wait for a change in the trend in response to an adjustment in feed, by the practice of what may be termed closed circuit thickening, which is accomplished through the use of the arrangement for recirculating the underflow. To this end, a portion of the underflow is returned from the surge tank to the thickener by way of flow line 49 and the return feed well 30 from which it is conducted to one or more different zones in the thickener through one or more of the different pipes 31, 32 or 33 controlled by valves 36, 34 and 35 respectively, according to what constituent is needed in the underflow.
- For example, if the underflow is medium or normal, the valves 34 and 35 are maintained closed and the valve 36 opened so as to direct the return from surge tank 38 through flow line 49, valve 36 and pipe 31 to a zone in the thickener near the central point of thickener discharge, whereby the character of the discharge is unchanged due to the fact that in this zone the composition of the material is the same as that being returned.
- If the underflow is low in lime, then valves 34 and 36 are maintained closed and valve 35 opened to feed the return from feed well 30 through valve 35 and pipe 33 to an intermediate zone of relatively high lime constituent, thus displacing the high-lime mixture with low-lime mixture with the result that the movement of the displaced high-lime mixture toward the discharge is hastened, while at the same time the returned low-lime mixture is placed a little nearer to the incoming high-lime corrective feed.

On the other hand, if the underflow is too rich in lime, valves 35 and 36 are maintained closed and valve 34 opened to direct the return through valve 34 and pipe 32 to an upper zone of low-lime mixture, thus displacing the low-lime mixture, with a high-lime mixture, with the result that the movement of the displaced low-lime mixture toward the discharge is hastened, and at the same time the returned high-lime mixture is placed near the incoming low-lime corrective feed, thus fastening equalization.

The number of return feed pipes such as 31, 32 and 33, and the location of the zones in the thickener to which they distribute the return feed, may be varied according to the location of the different zones of variation in mixture, the shape and proportions of the thickener, and the character of raw materials used.

From the surge tank 38, the underflow is passed via flow line 40 to one of the batch slurry mixers, say 43, the valve 41 being opened and the valve 42 closed for this purpose. When desired, the slurry passing into the slurry mixers may be sampled at some point in the flow line 40 as at 52 instead of or in addition to the catch samples taken at the surge tank 38. Final correction for obtaining the final desired complex ratios, if necessary, is accomplished in the slurry mixer by addition of the proper amount and kinds of correction materials, as indicated at 55, in a manner well understood by those skilled in the art. After the slurry mixer 43 is filled, the valve 41 is closed and the valve 45 opened to feed the contents of the mixer to the equalizing storage tank 47, while the supply of slurry from the surge tank is diverted to the next slurry mixer 44 and so on according to the number of slurry mixers used. From the storage tank 47 the mixture is fed through flow line 48 to the kilns, not shown, either

directly or first through a suitable filter or other suitable further dewatering device.

The long period of settling in the thickener with the substantial storage of settled slurry that is carried above the discharge point in the thickener gives a discharge moisture that is substantially free from variation as long as the average settling character of the raw materials remains constant. Where the settling character of the raw materials changes, the swing of moisture in the thickener discharge is very gradual permitting reliable readjustment of slurry feeders or filters ahead of the kiln so that constant tonnage rates through the kiln can be maintained. Even if the feeders or filters are not readjusted, the change is so gradual that conditions of irregular depth of charge in different parts of the kiln at the same time are avoided and a uniformly burned clinker can be obtained.

It will be understood that the system or plant and its operation as above described is not dependent on the specific elementary components falling strictly within the definitions used in the description for the sake of disclosure, for example, the term "flow line" is used to indicate any known or other suitable form of means or arrangement for conducting, guiding or conveying material from one point to another, such as a pipe, trough, conveyor, etc., according to the nature of the material conveyed and other exigencies of the particular phase in the process. Also the term valve is used to indicate any known or other suitable means for controlling the flow of material such as any known form of valve, stopper, gate or the equivalent selected according to the kind of conductor or conveyer in which it is used and the nature of the material whose flow is to be controlled.

The above described system of composition control is in practice substantially a one point control system, because the sampling and control of the thickener feed is the only one essential outside of the occasional checking of the trend of underflow composition and its correction locally by manipulation of the recirculation through the thickener pending response to control of the thickener feed.

Referring now to Fig. 2, this shows a modification using two relatively small equalizing storage thickeners 70 and 71 instead of a single relatively large thickener. The grinding is here shown as of the single stage type, but it is to be understood that it may also be of the double stage type as shown in Fig. 1. Here the raw materials are stored in high-lime and low-lime bins 72 and 73 respectively, according to their composition, which bins are arranged to supply the materials in proper controlled ratio, over flow line 74 to the mill 75. A Dorr bowl-classifier 76 is arranged in closed circuit with the mill 75 through flow lines 77 and 78, with its overflow discharging through flow line 79 to the equalizing storage thickeners 70-71, an automatic sampler 80 of any known or other suitable type being operatively associated with the flow line 79 for taking composite samples therefrom. The flow line 79 feeds the thickeners through branch lines 81 and 82 provided with suitable valve elements 83 and 84. Overflow from the thickeners is returned to the bowl classifier overflow line 85. Underflow from thickeners 70 and 71 is conducted over suitable flow lines 86 and 87 respectively, to several small, preferably 8-hour correction tanks 88, 89 and 90, selective distribution to the tanks being effected through branch conduits 91,

92, etc., controlled by valve elements 97, 98, etc. Conduits 103, etc., provided with suitable valve elements 106, etc., are arranged to conduct the slurry to the equalizing storage tank 109 from which the slurry is drawn as needed by way of a draw-off conduit 110 to a suitable kiln or kilns not shown. To afford knowledge of the composition of the slurry delivered through the underflow lines 86 and 87 of the thickeners, for proper proportioning of the fill in the correction tanks, these lines are provided with suitable sampling devices 111 and 112 operatively associated therewith. In carrying out the method of control with the system just described above, the bowl classifier overflow is diverted from flow line 79 over flow line 81 or 82 to high-lime thickener 70 or low-lime thickener 71, respectively, according as to whether the analyses of the samples taken at 80 indicate the overflow to be of high lime content or low lime content. The thickened slurry is drawn from both thickeners 70 and 71 into the correction tanks 88 etc., to fill them with mixture of the desired composition, which composition is controlled by proper proportioning of the mixtures, furnished by the different thickeners in accordance with the lime content of such mixtures shown by analyses of the samples taken at 111 and 112. Advantage is taken of the inherent equalizing effect of the thickeners to insure against substantial change in composition of thickener underflow in the time interval between the sampling and analyzing, with the result that a very fine control of the composition 35 of the mixture in the correction tanks is accomplished.

From the correction tanks the slurry is passed to the usual equalizing storage 109 from whence it is fed as required over flow line 110 to suitable kilns not shown. To enhance the equalizing effect of the thickeners they may be operated periodically as slurry mixers by driving the rakes at relatively higher speed, preferably so operating one when the other is receiving all or substantially all of the feed.

Where the high-lime and low-lime thickeners are of a size sufficient only to handle a portion of total feed from the bowl classifier overflow, for example 75 per cent, the arrangement of Fig. 50 3 is used, wherein the overflow, after passing the sampler is caused to flow through a suitable splitter 125 to split the feed to the thickeners in the ratio of 25 per cent to the low-lime thickener 71 and 75 per cent to the high-lime thickener 70, 55 when the analyses of the samples indicates a high lime content, and in the opposite ratio when the analysis indicates a low lime content.

Where it is desired to use a still larger number of smaller thickeners, say three, each of a capacity sufficient only to handle say 50 per cent of the total overflow from the bowl classifier, the arrangement shown in Fig. 4 is used wherein the overflow from the bowl classifier after passing the sampler is arranged to be diverted to either 65 of the flow lines 126 or 127 by means of suitable valve elements 128 and 129, according as to whether the analyses of the samples indicate a high-lime content or a low-lime content respectively. The flow line 126 is arranged to conduct the feed through a suitable splitter 130 to both the high-lime thickener 70 and a tertiary or medium-mixture thickener 132, the splitter being arranged to divide the feed equally between the two thickeners. The flow line 127 is similarly 70 arranged to conduct the feed through a suitable 75

splitter 131 in equal proportions to the low-lime thickener 71 and the medium-mixture thickener 132. In operation, when the analyses taken at the sampler indicate a high lime content, the valve element 129 is closed and the valve element 128 opened to divert the feed overflow line 126 and through splitter 130 in equal proportions to the thickeners 70 and 132. Likewise, when the analyses indicate a low lime content valve element 128 is closed and 129 opened to divert the feed through flow line 127 and splitter 131, in equal proportions to thickeners 71 and 132. 10

The three thickeners will thus serve as equalizing storage zones for the mixtures of three different characters, high lime, low lime, and medium, from which the underflow may be drawn in proper proportions for mixtures in the usual suitable correction tanks, in a manner which will be well understood in the light of the description of Fig. 2 up to step 20 above 20

It will be clear from the above that this phase of the invention involving the splitting of the feed in different proportions to different thickeners will be varied in its application according to the capacity of the thickeners in relation to the volume of feed supply. For example, where three thickeners are used, each of a capacity less than 50 per cent of the total supply, a three way splitter would be used, arranged to divide as much of the feed as can be handled by two thickeners, 30 equally between one of the extreme thickeners and the tertiary thickener, diverting the small remainder to the other extreme thickener, the distribution being alternated in relation to the extreme thickeners according to variations in the lime content of the feed. A modification of this latter system of feed is to feed one of the extreme thickeners at full capacity (less than half the total supply) and distribute the remainder of the supply equally between the two remaining thickeners. 35

While certain specific modifications, embodiments and applications of the invention have been herein shown and described for the purpose of disclosure, it is to be understood that the invention is not limited to such specific embodiments and applications, but contemplates all such modifications and variants thereof as fall fairly within the scope of the appended claims. 45

Having thus described the invention what is 50 claimed and desired to be secured by Letters Patent is:

1. In the process of manufacturing cement by wet grinding, the method of controlling the composition of the finished ground mixture to be burned, which comprises passing the finished ground material into a settling zone, withdrawing a portion of the settled mixture for said burning, analyzing a sample of the portion withdrawn for burning, and returning to the settling zone a portion of the mixture withdrawn, to displace a portion of the mixture in the settling zone having an excess of the element needed in the sample tested. 55

2. In the process of manufacturing cement by wet grinding, the method of controlling the composition of the finished ground mixture to be burned, which comprises passing the finished ground mixture into a settling zone, withdrawing a portion of the settled mixture for said burning, analyzing a sample of the portion withdrawn for burning, and using a portion of the mixture withdrawn to displace portions of those strata in the settling zone containing a corrective mixture and thereby accel- 70 75

erating the movement of the displaced portion toward the point of discharge. 1,985,868  
3. In a process of manufacturing cement including a step at which the ground raw mixture of given desired composition is detained in relatively large volume, and portions thereof withdrawn from the zone of detention; the method of varying the composition of the mixture withdrawn from the zone of detention which comprises displacing portions of the mixture in the zone of detention having an excess of the element wanting in the mixture withdrawn with portion of the mixture withdrawn to disturb the stratification of portions of different composition in the zone of detention. 1,985,868  
4. In a process of manufacturing cement including a step at which the ground raw mixture of given desired composition is detained in relatively large volume, and portions thereof withdrawn from the zone of detention; the method of controlling the composition withdrawn from the zone of detention which comprises using a portion of the mixture withdrawn to displace portions of those strata containing a corrective mixture and thereby accelerate the movement of such portions toward the point of discharge. 1,985,868  
5. The process of making cement which comprises segregating the raw material into high-lime and low-lime supplies, proportioning a mixture of the said supplies to form a grinding mill feed, grinding the mill feed, hydraulically classifying the mill discharge, passing the classifier overflow to a thickener, sampling and analyzing the classifier overflow, sampling the thickener discharge, varying the said mixture of raw materials to vary the composition of the classifier

overflow as indicated by the analysis of such overflow to compensate for variation in the thickener discharge as indicated by the analysis thereof, and accelerating the movement of certain high-lime or low-lime portions of the thickener contents toward the discharge to correct composition of discharge during time required to effect correction of thickener contents by variation of raw material composition, by returning or recirculating thickener underflow to certain sludge zones in the thickener in a manner substantially as described. 1,985,868

6. In the manufacture of cement by wet grinding, the method of controlling the composition of the finished ground mixture to be burned, which comprises passing the finished ground mixture into a settling zone at a dilution greater than that of the mill discharge, repeatedly diverting a portion of the feed in its passage to the settling zone and analyzing said sample, varying the composition of the feed to compensate for any variation from the desired composition as indicated by such analyses, withdrawing the settled mixture from the settling zone for burning, sampling and analyzing the mixture withdrawn, and controlling the composition of the mixture withdrawn to compensate for fluctuations in the composition of the feed by returning to the settling zone a portion of the mixture withdrawn to displace other portions of the mixture in the settling zone such as are rich in the element wanting in the mixture withdrawn to accelerate the movement of such displaced portions to the point of discharge. 1,985,868

ERNEST J. MAUST.